

# UNITED STATES PATENT OFFICE.

WILLIAM JONES, OF LONDON, ENGLAND, ASSIGNOR OF ONE-HALF TO  
RICHARD CHARLES POWELL, OF SAME PLACE.

## TRANSFER-SHEET.

SPECIFICATION forming part of Letters Patent No. 369,795, dated September 13, 1887.

Application filed August 28, 1886. Serial No. 212,119. (No model.)

*To all whom it may concern:*

Be it known that I, WILLIAM JONES, a subject of the Queen of England, residing at London, England, map-mount, have invented 5 certain new and useful Improvements in or relating to the Preparation of Transfer-Sheets, of which the following is a specification.

In carrying out my invention I use a "sheet" composed of "tracing-tissue," newspaper, 10 cloth, or other suitable substance, and coat it on both sides with a varnish composed of the following ingredients, viz: two parts, by measurement, of white spirit-varnish; two parts methylated spirits; one part turpentine; one 15 part castor-oil, the whole to be thinned down with paraffine or other mineral oil, and, by preference, scented with verbena or other essential oil. The paper or cloth having its surfaces coated with the above varnish is then 20 pressed and covered on one side with spirit-varnish and backed in the other with one or more layers of cartridge, drawing, printing, or lithographic paper, or other suitable strengthening material, attached by means of starch or 25 other adhesive material and again pressed. The surface of the tracing-tissue or newspaper or textile fabric is then covered or faced with an "enamel" consisting of gelatine-glue and glycerine, the enamel known as "Cory's mountain snow" or other enamel, and again rolled 30 or pressed and allowed to dry, when the enamelled surface is ready to receive the picture, design, or print, which may be applied in the usual manner. The sheet I employ thus consists of an enamel face applied to a "body" of 35 "tissue" of fine quality supported by a stronger backing.

To produce a transparency, the printed or ornamented face of the "material" is attached 40 to glass by a mixture of gum and alum or other adhesive material, being well pressed thereon and all air-bubbles being removed by means of a "squeegee," in the manner usually practiced by those skilled in the art of mounting 45 prints or drawings. After the adhesive material has had time to dry—a process which usually requires about a day—the backing is

moistened with glycerine and water, and, if proper care be taken, the backing and also the tracing-tissue or body can be removed sheet 50 by sheet until nothing remains upon the glass but the enameled face bearing the color or impression. When the desired degree of attenuation or transparency has been arrived at, the transferred picture may be either coated on 55 the back with a protective varnish or it may be French polished or protected by glass.

When it is required to apply the print or design to non-transparent surfaces—such as 60 china or opaque glass—it is fixed thereon by means of a volatile or combustible varnish. The body and backing are then removed, as above described, leaving the film of color and enamel, and the china or glass is then fired in the usual manner.

I do not confine myself to the precise proportions of the ingredients which I have herein mentioned, although I find these to give satisfactory results.

I claim—

1. As a new article of manufacture, a transfer-sheet consisting of a body material of tracing-linen or other suitable tissue, provided with an enamel coating on its face side, and a 75 backing of paper or other textile or fibrous material stronger than the body, substantially as specified.

2. The process herein described of making transfer-sheets, which consists in the employment of a sheet of tracing-linen or other suitable tissue as the body material, varnishing the same on both sides, then covering one side with an enamel and attaching to the other side a backing of stout paper or other textile or fibrous material of a stronger character than 80 the body, substantially as set forth.

In testimony whereof I have hereto set my hand in the presence of two subscribing witnesses.

WILLIAM JONES.

Witnesses:

ALFRED J. BOULT,  
HARRY B. BRIDGE.